# EUROPEAN PATENT SPECIFICATION

(11) **EP 0 770 122 B1**
(45) Date of publication and mention of the grant of the patent: **09.12.1998**
(21) Application number: 95925829.4
(22) Date of filing: 05.07.1995
(51) Int. Cl.: C11D 3/37

(54) **STABLE, AQUEOUS CONCENTRATED LIQUID DETERGENT COMPOSITIONS CONTAINING HYDROPHILIC COPOLYMERS**
STABILE WÄSSRIGE KONZENTRIERTE FLÜSSIGWASCHMITTEL ENTHALTEND HYDROPHILE COPOLYMERE
COMPOSITIONS DETERGENTES LIQUIDES CONCENTREES AQUEUSES STABLES, CONTENANT DES COPOLYMERES HYDROPHILES

(30) Priority: 14.07.1994 US 274948; 14.07.1994 US 274938
(43) Date of publication of application: 02.05.1997
(73) Proprietor: BASF CORPORATION, Mount Olive, New Jersey 07828-1234 (US); BASF AKTIENGESELLSCHAFT, 67056 Ludwigshafen (DE)
(72) Inventor: GOPALKRISHNAN, Sridhar, Woodhaven, MI 48183 (US); SHERMAN, John, V., Allen Park, MI 48101 (US); GUINEY, Kathleen, M., Wyandotte, MI 48192 (US); DUROCHER, David, T., Westland, MI 48185 (US); WELCH, Michael, C., Woodhaven, MI 48183 (US)
(74) Representative: Stark, Vera, Dr.
(86) International application number: EP9502597
(87) International publication number: WO9602622

(56) References cited:
- EP-A- 0 543 562
- FR-A- 2 677 655
- GB-A- 2 256 646
- US-A- 4 797 223
- PATENT ABSTRACTS OF JAPAN vol. 007 no. 077 (C-159) ,30 March 1983 & JP,A,58 007415 (NIPPON SHOKUBAI KAGAKU KOGYO KK) 17 January 1983,

## Description

### FIELD OF THE INVENTION

The present invention relates to hydrophilic copolymers, and more particularly, to stable, aqueous-based, concentrated liquid detergents that contain the hydrophilic copolymers and thus permit the incorporation of builders, polymers and other water- insoluble components to form a stable composition. The invention also relates to a method of stabilizing liquid detergent compositions.

### BACKGROUND OF THE INVENTION

The incorporation of major amounts of builders in liquid detergent compositions poses a significant formulating challenge since the presence of major amounts of builder inevitably causes the detergent composition to phase separate. Builders such as sodium citrate, citric acid, sodium carbonate, and/or alkali metal silicates can only be incorporated in minor amounts in liquid detergent compositions, such amounts being typically below the concentration levels that would cause separation of the surfactant phase. Liquid detergent formulations that contain builders thus require careful control of the surfactant to builder ratio so as to prevent "salting-out" of the surfactant phase. The literature is replete with examples of such compositions.

Montague, U.S. Patent No. 5,147,576, relates to detergent compositions that comprise a relatively high amount of detergent active matter and further allow the incorporation of builders and suspension of particulate solids. Such compositions are prepared by adding an electrolyte/builder to the surfactant rich aqueous phase so as to result in a structure of lamellar droplets dispersed in the continuous aqueous phase. These compositions also require the incorporation of a minor amount of a "deflocculating polymer" in the detergent composition. The deflocculating polymer, according to this reference, is required to comprise of a hydrophilic backbone with at least one hydrophobic side chain. The preparation of such polymers are accomplished by copolymerizing hydrophilic monomers with a hydrophobic monomer. The hydrophobic monomer contains a hydrophobic side chain. The polymerization of the hydrophilic monomer and the hydrophobic monomer is conducted in a cosolvent, which is typically water and another solvent in which the hydrophobic monomer is soluble.

### OBJECTS OF THE INVENTION

It is therefore an object of the present invention to incorporate a hydrophilic copolymer into a liquid detergent composition which will impart stability to the detergent over extended periods of storage.

Another object of the present invention is to provide an aqueous-based laundry detergent formulation which has significant amounts of detergent active matter and builders which shows virtually no phase separation.

A further object of the invention is to provide a novel, hydrophilic copolymer useful in stabilizing liquid laundry detergents.

Another object is to provide a method of stabilizing laundry formulations.

### SUMMARY OF THE INVENTION

These and other objects of the invention are achieved by providing a stable liquid detergent composition, comprising:
a) 5 - 70% of detergent active matter selected from the group consisting of anionic, nonionic, cationic, amphoteric and zwitterionic surfactants;
b) 1 - 60% of one or more electrolytes;
c) 0.01 - 5% of at least one hydrophilic copolymer containing randomly distributed within the polymer backbone units represented by formula I or II where x, y, z, a, and b are integers and M is a alkali metal such as sodium, or hydrogen, (x + y):z is from 5:1 to 1000:1, and y can be any value ranging from zero up to the maximum value of x and b can be zero
   R₁ = H or CH₃
   R₂ = COOM, OCH₃, SO₃M, O-CO-CH₃, CO-NH₂
   R₃ = CH₂-O-, CO-NH-
   R₄ = -CH₂-CH₂-O
   R₅ = alkyleneoxy group, preferably propyleneoxy or butyleneoxy groups, with the provision that the values of a and b in the sidechain are such that the combined weights of R₄ and R₅ are such that the monomer has a solubility of at least 500 grams/liter in water at 20°C;
   Where R₆ = or mixtures of both, wherein in Formula II, x, y, z, a, and b are integers and M is an alkali metal such as sodium, or hydrogen, (x + y):z is from 5:1 to 1000:1, and y can be any value ranging from zero up to the maximum value of x, and b can be zero
   R₃ = H or CH₃
   R₂ =COOM, OCH₃, SO₃M, O-CO-CH₃, CO-NH₂
   R₄ is ethyleneoxy and R₅ is alkyleneoxy, preferably propyleneoxy or butyleneoxy, with the provision that, if b is different from zero, the values of a and b in the sidechain are such that the combined weights of R₄ and R₅ are such that the monomer has a solubility of at least 500 grams/liter in water at 20°C; and
d) water; said composition having a phase separation of less than 2% over a one month period.

Also provided as part of the invention is a method of stabilizing a liquid detergent composition which comprises adding 0.01 - 5% by weight of at least one hydrophilic copolymer containing randomly distributed within the polymer backbone units represented by formula I or II where x, y, z, a, and b are integers and M is a alkali metal, or hydrogen, (x + y):z is from 5:1 to 1000:1, and y can be any value ranging from zero up to the maximum value of x and b can be zero
R₁ = H or CH₃
R₂ = COOM, OCH₃, SO₃M, O-CO-CH₃, CO-NH₂
R₃ = CH₂-O-, CO-NH-
R₄ = -CH₂-CH₂-O
R₅ = alkyleneoxy group, preferably propyleneoxy or butyleneoxy groups, with the provision that, if b is different from zero, the values of a and b in the sidechain are such that the combined weights of R₄ and R₅ are such that the monomer has a solubility of at least 500 grams/liter in water at 20°C;
where R₆ = or mixtures of both; wherein in Formula II, x, y, z, a, and b are integers and M is a alkali metal such as sodium, or hydrogen, (x + y):z is from 5:1 to 1000:1, and y can be any value ranging from zero up to the maximum value of x, and b can be zero
R₁ = H or CH₃
R₂ = COOM, OCH₃, SO₃M, O-CO-CH₃, CO-NH₂
R₄ is ethyleneoxy and R₅ is alkyleneoxy, preferably propyleneoxy or butyleneoxy, with the provision that, if b is different from zero, the values of a and b in the sidechain are such that the combined weights of R₄ and R₅ are such that the monomer has a solubility of at least 500 grams/liter in water at 20°C.

### DETAILED DESCRIPTION OF THE PREFERRED EMBODIMENT

The hydrophilic copolymer of the invention is represented by Formula I or II: Where x, y, z, a, and b are integers and M is a alkali metal, or
hydrogen and the monomer units are in random order, (x + y):z is from 5:1 to 1000:1, and y can be any value ranging from zero up to the maximum value of x, and b can be zero.
R₁ = H or CH₃
R₂ =COOM, OCH₃, SO₃M, O-CO-CH₃, CO-NH₂
R₃ = CH₂-O-, CH₂-N-, COO-, -O-, CO-NH-
R₄ = -CH₂-CH₂-O
R₅ = alkykeneoxy group, preferably propyleneoxy or butyleneoxy groups, with the provision that, if b is different from zero,
the values of a and b in the sidechain are such the combined weights of R₄ and R₅ are such that the monomer has a solubility of at least 500 grams/liter in water at 20°C

Where R₆ = or mixtures of both. In Formula II, x, y, z, a, and b are integers and M is a alkali metal, or hydrogen and the monomer units are in random order, (x + y):z is from 5:1 to 1000:1, and y can be any value ranging from zero up to the maximum value of x, and b can be zero and
R₁ = H or CH₃
R₂ = COOM, OCH₃, SO₃M, O-CO-CH₃, CO-NH₂
R₄ is ethyleneoxy and R₅ is alkyleneoxy, preferably propyleneoxy or butyleneoxy, with the provision that, if b is different from zero, the values of a and b in the sidechain are such the combined weights of R₄ and R₅ are such that the monomer has a solubility of at least 500 grams/liter in water. It is within the scope of the invention that R₄ and R₅ be interchangeable in the sidechain.

As heretofore stated, the molar ratio of x + y to z in both Formulas I and II is within the range of 5:1 to 1000:1, preferably 50:1 to 800:1, and more preferably 100:1 to 500:1. If b is zero, the value of a is preferably within the range of 1 to 200, more preferably 1 to 150, and more preferably 1 to 100.

The total molecular weight of the copolymer will be within the range of 500 to 500,000, as determined by gel permeation chromatography. It is further desirable that the molecular weight fall within the range of 1,000 to 100,000, and even more preferably be within the range of 1,000 to 10,000 (weight average molecular weight - WAMW; unless otherwise specified, molecular weights herein are given in terms of WAMW).

The hydrophilic copolymers of the present invention are prepared by copolymerizing two hydrophilic monomers, an unsaturated hydrophilic monomer copolymerized with an oxyalkylated monomer. These monomers may be randomly distributed within the polymer backbone. Preparation of oxyalkylated monomers could be carried out in accordance with Tang, U.S. Patent No. 5,162,475, incorporated herein by reference. In Tang, Example 1 is especially relevant. Gosselink, U.S. Patent No. 4,622,378, is also relevant, and is also incorporated herein.

The unsaturated hydrophilic monomer may be selected from the group consisting of acrylic acid, maleic acid, maleic anhydride, methacrylic acid, methacrylate eaters and substituted methacrylate esters, vinyl acetate, as well as vinyl acetate copolymerized with said oxyalkylated monomer and hydrolyzed to polyvinyl alcohol, methylvinyl ether, and vinylsulphonate. Preferably, the unsaturated hydrophilic monomer component of the hydrophilic copolymer in formula I or II is acrylic acid. Other useful monomers will include crotonic acid, itaconic acid, as well as vinyl acetic acid.

Examples of the oxyalkylated monomer would be compounds that have a polymerizable olefinic moiety with at least one acidic hydrogen and are capable of undergoing addition reaction with alkylene oxides. It is also possible to include monomers with at least one acidic hydrogen that are polymerized first, and then subsequently oxyalkylated to yield the desired product. For example, allyl alcohol is especially preferred since it represents a monofunctional initiator with a polymerizable olefinic moiety having an acidic hydrogen on the oxygen, and is capable of adding to alkylene oxide. Similarly diallylamine represents another monofunctional initiator with polymerizable olefinic moieties, having an acidic hydrogen on the nitrogen, and is capable of adding to alkylene oxide. Other examples of the oxyalkylated monomer of the copolymer will include reaction products of either acrylic acid, methacrylic acid, maleic acid, or 3-allyloxy-1,2-propanediol with alkylene oxide, preferably ethylene oxide.

The molecular weight of the oxyethylated monomer in formula I or II (in both cases b = 0) according to the various embodiments of the invention will be within the range of 200 to 30,000, more preferably 500 to 15,000, and even more preferably 1000 to 5000.

The oxyethylated moiety represents the side chain of this monomer. The side chain is hydrophilic in nature, that is, the side chain when isolated from its linkage to the backbone carbon atom is completely soluble in water. The monomer unit containing the hydrophilic side chain also has similar solubility characteristics as the side chain. Preferably, the side chain when isolated from its linkage to the backbone will have a solubility in water of at least 700 grams/liter, and even more preferably 1000 grams/liter, or more. Moreover, the entire side chain is hydrophilic in nature by virtue of its extensive solubility in water.

The hydrophilic copolymer as part of the invention may be prepared by the skilled artisan according to the process below, in which the ethylene oxide adduct of allyl alcohol is copolymerized with acrylic acid by way of a non-limiting example.

### Preparation of Ethylene Oxide Adduct of Allyl Alcohol (A)

- To a 3.785 l (1 gallon) stainless steel autoclave equipped with steam heat, vacuum and nitrogen pressure capability and agitation, a homogenous mixture of 210.5 grams of allyl alcohol and 23.4 grams of potassium t-butoxide was charged. The vessel was sealed, purged with nitrogen and pressurized to 6.3 bar (90 psig) with nitrogen. The pressure was then readjusted to 2.38 bar (34 psig) and the temperature of the vessel was adjusted to 80°C. The first 75 grams of ethylene oxide was charged over a 1 hour period at 75 - 85°C and < 6.3 bar (< 90 psig) pressure. The next 125 grams of ethylene oxide was charged over an hour period at 75 - 85°C and < 6.3 bar (< 90 psig). The next 225 grams of ethylene oxide was charged over a 1 hour period at 100 - 110°C and < 6.3 bar (< 90 psig). The remaining 2140.9 grams of ethylene oxide was added over an 8 hour period at 145 - 155°C and < 6.3 bar (< 90 psig) pressure. After all of the ethylene oxide was added, the mixture was reacted at 150°C for 2 hours and the vessel was vented to 0 psig. The material was stripped at < 10 mm Hg and 125°C for 1 hour then cooled to 50°C and discharged into an intermediate holding tank for analysis.

To a 7.57 l (2 gallon) stainless steel autoclave equipped with steam heat, vacuum, nitrogen pressure capability and agitation, 498.8 grams of the allyl alcohol ethylene oxide intermediate was charged. The vessel was sealed and pressurized to 6.3 bar (90 psig) with nitrogen and vented to 0.14 bar (2 psig). This was repeated two more times. The temperature was adjusted to 145°C and the pressure was readjusted to 2.38 bar (34 psig) with nitrogen. To the vessel, 2198.3 grams of ethylene oxide was charged at 275 grams per hour. The temperature was maintained at 140 - 150°C and the pressure was maintained at < 90 psig. If the pressure rose above 5.95 bar (85 psig), the ethylene oxide addition was slowed. If this failed to lower the pressure, the addition was halted and allowed to react at 145°C for 30 minutes. The vessel was slowly vented to a 0 psig and repadded to 2.38 bar (34 psig) with nitrogen. The addition was continued at 140 - 150°C and < 6.3 bar (< 90 psig) pressure. After all of the ethylene oxide was added, the material was held at 145°C for 1 hour. It was then cooled to 900 and 2.9 grams of 85% phosphoric acid was added. The material was mixed for 30 minutes and then vacuum stripped at 100°C for 1 hour. The batch was cooled to 70°C and discharged into a holding tank. The product was found to have a number average molecular weight of 4095 g/mol by phthalic anhydride esterification in pyridine.

### Copolymerization of Monomer A with Acrylic Acid

To a two liter, four-necked flask equipped with a mechanical stirrer, reflux condenser, thermometer, and outlet for feed lines, were added 301 grams of distilled water and 2.6 grams of 70% phosphorous acid. This solution was heated to 95°C at which time a monomer blend of 555.4 grams of glacial acrylic acid and 62.8 grams of an allyl alcohol initiated ethoxylate (molecular weight ~ 3800), a redox initiator system consisting of 132 grams of a 38% sodium bisulfite solution and 155.2 grams of a 10.9% sodium persulfate solution, are fed into the flask linearly and separately while maintaining the temperature at 95 (+/-3)°C. The sodium bisulfite solution and monomer blend feeds are added over 4 hours while the sodium persulfate solution is added over 4.25 hours. The three feeds are added via TEFLON · 1/8 inch tubing lines connected to rotating piston pumps. Appropriately sized glass reservoirs attached to the pumps hold the monomer blend and initiator feeds on balances accurate to 0.1 gram to precisely maintain feed rates. When the additions are complete, the system is cooled to 80°C. At this temperature, 25.3 grams of a 2.4% 2,2'-Azobis(N,N'-dimethyleneisobutylramidine)dihydrochloride solution is added to the system over 0.5 hours as a postpolymerizer. When addition is complete the system is reacted for 2 hours at 80°C. After reaction, the system is cooled to 60°C and the solution pH is adjusted to about 7 with the addition of 658 grams of 50% sodium hydroxide solution. The resultant neutral polymer solution has an approximate solids content of about 40%.

Especially preferred is the oxyalkylated monomer which is a propylene oxide and ethylene oxide adduct of allyl alcohol. This monomer has a molecular weight of about 3800, and R₄ is a propyleneoxy group represented by the formula -CH₂-CH(CH₃)-O and R₅ is -CH₂-CH₂-O. In this monomer, R₁ = H, R₂ = COOM, R₃ = CH₂ - O, and y = O, M is sodium in this monomer as well.

The weight ratio of R₄ : R₅ in the oxyalkylated monomer is preferably about 1:4 (this ratio may vary considerably, so long as the solubility criteria of at least 500 grams/liter is met).

The molecular weight of the oxyalkylated monomer according to the various embodiments of the invention will be within the range of 200 to 30,000, more preferably 500 to 15,000, and more preferably 1000 to 5000.

The oxyalkylated moiety represents the side chain of this monomer. The side chain is hydrophilic in nature, that is, the side chain when isolated from its linkage to the backbone carbon atom has extensive solubility in water. The monomer unit containing the hydrophilic side chain also has similar solubility characteristics as the side chain. Preferably, the side chain when isolated from its linkage to the backbone will have a solubility in water of at least about 500 grams/liter, and even more preferably about 700 grams/liter, or more. Moreover, the entire side chain is hydrophilic in nature by virtue of its extensive solubility in water.

The hydrophilic copolymer as part of the invention may be prepared by the skilled artisan according to he process below, in which the alkylene oxide adduct of allyl alcohol is copolymerized with acrylic acid by way of a non-limiting example.

### Preparation of Alkylene Oxide Adduct of Allyl Alcohol (Monomer B)

To a 7.57 l (2 gallon) stainless steel autoclave equipped with steam heat, vacuum and nitrogen pressure capability and agitation, a homogenous mixture of 396.2 grams of allyl alcohol and 44.1 grams of potassium t-butoxide was charged. The vessel was sealed, purged with nitrogen and pressurized to 6.3 bar (90 psig) with nitrogen. The pressure was then relieved to 0.14 bar (2 psig) and the temperature of the vessel was adjusted to 80°C. The first 125 grams of propylene oxide was added over a 1 hour period. The temperature was maintained between 75 - 85°C and the pressure was maintained at < 6.3 bar (<90 psig). The next 200 grams of propylene oxide was added over a 1 hour period and at 75 - 85°C and < 6.3 bar (<90 psig) pressure. The next 400 grams of propylene oxide was added over a 1 hour period at 100-110°C and < 6.3 bar (<90 psig) pressure. The remaining 4551.2 grams of propylene oxide was charged at 500 grams per hour and at 120-130°C and < 6.3 bar (<90 psig) pressure. After all of the propylene oxide was added, the mixture was reacted at 125°C for 2 hours and the vessel was vented to 0 psig. The material was stripped at <10mm Hg and 125*C for 1 hour then cooled to 50°C and discharged into an intermediate holding tank for analysis.

To a 18.925 l (5 gallon) stainless autoclave equipped with steam heat, vacuum and nitrogen pressure capability and agitation, 2696.8 grams of the allyl alcohol propylene oxide intermediate was charged. The vessel was sealed and pressurized to 6.3 bar (90 psig) with nitrogen and vented to 0.14 bar (2 psig). This was repeated two more times. The temperature was adjusted to 145°C and the pressure was readjusted to 2.38 bar (34 psig) with nitrogen. To the vessel, 10788.9 grams of ethylene oxide was charged at 1400 grams per hour. The temperature was maintained at 140-150*C and the pressure was maintained at < 6.3 bar (<90 psig). If the pressure rose above 5.95 bar (85 psig), the ethylene oxide addition was slowed. If this failed to lower the pressure, the addition was halted and allowed to react at 145°C for 30 minutes. The vessel was slowly vented to 0 psig and repadded to 2.38 bar (34 psig) with nitrogen. The addition was continued at 140-150°C and 6.3 bar (<90 psig) pressure.

After all of the ethylene oxide was added, the material was held at 145°C for 1 hour. It was then cooled to 90°C and 14.3 grams of 85% phosphoric acid was added. The material was mixed for 30 minutes and then vacuum stripped at 100°C for 1 hour. The batch was cooled to 70°C and discharged into a holding tank. The product was found to have a number average molecular weight of 4091 by phthalic anhydride esterification in pyridine.

### Polymerization of Monomer B with Acrylic Acid

To a two liter, four necked flask equipped with a mechanical stirrer, reflux condenser, thermometer, and outlet for feed lines, were added 301 grams of distilled water and 2.6 grams of 70% phosphorous acid. This solution was heated to 95 degrees centigrade at which time a monomer blend of 555.4 grams of glacial acrylic acid and 61.7 grams of an allyl alcohol initiated propoxylate ethoxylate (B) (molecular weight 3500), a redox initiator system consisting of 132 grams of a 38% sodium bisulfite solution and 155.4 grams of a 10.9 % sodium persulfate solution, are fed into the flask linearly and separately while maintaining the temperature at 95 + or - 3 degrees centigrade. The sodium bisulfite solution and monomer blend feeds are added cver 4 hours while the sodium persulfate solution is added over 4.25 hours. The three feeds are added via teflon 1/8 inch tubing lines connected to rotating piston pumps. Appropriately sized glass reservoirs attached to the pumps hold the monomer blend and initiator feeds on balances accurate to 0.1 gram to precisely maintain feed rates. When the additions are complete, the system is cooled to 80 degrees centigrade. At 80 degrees centigrade, 25.3 grams of a 2.4% 2,2'-Azobis (N,N'-dimethyleneisobutyramidine) dihydrochloride solution is added to the system over 0.5 hours as a postpolymerizer. When addition is complete the system is reacted for 2 hours at 80 degrees centigrade. After reaction, the system is cooled to 60 degrees centigrade and the solution pH is adjusted to about 7 with the addition of 658 grams of 50% sodium hydroxide solution.

The resultant neutral polymer solution has an approximate solids content of 40%.

The hydrophilic copolymer of the invention is added to detergent compositions, hereinafter described, to impart stability thereto. For purposes of definition, stable detergent compositions are those that do not give more than about a 2% phase separation upon storage at room temperature for a period of one month (30 days) from the time of preparation. Preferably, the phase separation is within the range of about 0 - 2%, and even more preferably less than about 1%. The volume fraction of the separated aqueous phase is measured as a function of the total volume of the sample. For example, if the total volume of the sample is 100 ml, then a 2% separation would correspond to 2 ml.

The hydrophilic copolymer will therefore comprise about 0.01 to 5% by weight of the liquid detergent composition. Preferably, the copolymer of the invention will make up 0.5 to 4% of a typical laundry formulation, even more preferably 1 to 2%. (Unless otherwise stated, all weight percentages are based upon the weight of the total laundry formulation).

The laundry formulation will contain 5 to 70% of detergent active matter, more preferably 15 to 40%, and even more desirably greater than 25 and up to 35%.

The detergent active matter may be selected from the group of anionic, nonionic, cationic, amphoteric and zwitterionic surfactants known to the skilled artisan. Examples of these surfactants may be found in NcCutcheon, Detergents and Emulsifiers 1993, incorporated herein by reference. Examples of nonionic surfactants will include commonly utilized nonionic surfactants which are either linear or branched and have an HLB of from about 6 to 18, preferably from about 10 to 14. Examples of such nonionic detergents are alkylphenol oxyalkylates (preferably oxyethylates) and alcohol oxyethylates. Examples of the alkylphenol oxyalkylates include C₆-C₁₈-alkylphenols with 1 - 15 moles of ethylene oxide or propylene oxide or mixtures of both. Examples of alcohol oxyalkylates include C₆ - C₁₈ alcohols with 1 - 15 moles of ethylene oxide or propylene oxide or mixtures of both. Some of these types of nonionic surfactants are available from BASF Corp. under the trademark PLURAFAC. Other types of nonionic surfactants are available from Shell under the trademark NEODOL. In particular, a C₁₂ - C₁₅ alcohol with an average of 7 moles of ethylene oxide under the trademark NEODOL® 25-7 is especially useful in preparing the laundry detergent compositions useful in the invention. Other examples of nonionic surfactants include products made by condensation of ethylene oxide and propylene oxide with ethylene diamine (BASF, TETRONIC® and TETRONIC® R). Also included are condensation products of ethylene oxide and propylene oxide with ethylene glycol and propylene glycol (BASF, PLURONIC® and PLURONIC®R). Other nonionic surface active agents also include alkylpolyglycosides, long chain aliphatic tertiary amine oxides and phosphine oxides.

Typical anionic surfactants used in the detergency art include the synthetically derived water-soluble alkali metal salts of organic sulphates and sulphonates having 6 to 22 carbon atoms. The commonly used anionic surf actants are sodium alkylbenzene sulphonates, sodium alkylsulphates and sodium alkylether sulphates. Other examples include reaction products of fatty acids with isethionic acid and neutralized with sodium hydroxide, sulphate esters of higher alcohols derived from tallow or coconut oil, and alpha-methylestersulfonates.

Examples of amphoylitic detergents include straight or branched aliphatic derivatives of heterocyclic secondary or tertiary amines. The aliphatic portion of the molecule typically contains about 8 to 20 carbon atoms. zwitterionic detergents include derivatives of straight or branched aliphatic quaternary ammonium, phosphonium or sulfonium compounds.

The laundry detergent formulation will also contain one or more electrolytes. Electrolytes defined herein are any ionic water-soluble material. The presence of the electrolyte is often required to bring about the structuring of the detergent active material, although lamellar dispersions are reported to be formed with detergent active material alone in the absence of a suitable electrolyte. Electrolytes typically comprise from about 1 to 60% by weight, and more preferably about 25 to 35% of a laundry detergent formulation.

Examples of suitable electrolytes include compounds capable of providing sufficient ionic strength to the aqueous detergent composition. These compounds would include alkali metal salts of citric acid, alkali metal carbonates, and alkali metal hydroxides. Of these, sodium citrate, sodium carbonate and sodium hydroxide are preferred. Potassium salts can also be incorporated to promote better solubility. other examples of suitable electrolytes will include the phosphate salts such as sodium or potassium tripolyphosphate, and alkali metal silicates.

In many cases the electrolyte utilized will also serve as the builder for enhancing detergency. The builder material sequesters the free calcium or magnesium ions in water and promote better detergency. Additional benefits provided by the builder are increased alkalinity and soil suspending properties. With the near phase-out of phosphate in household laundry detergents, the most commonly used non-phosphate builders are the alkali metal citrates, carbonates, bicarbonates and silicates. All of these compounds are water-soluble. Water-insoluble builders which remove hardness ions from water by an ion-exchange mechanism are the crystalline or amorphous aluminosilicates referred to as zeolites. Mixtures of electrolytes or builders can also be employed. Generally, the amount of electrolyte used in laundry detergent compositions according to the invention will be well above the solubility limit of the electrolyte. Thus, it is possible to have undissolved electrolyte which remains suspended in the liquid matrix. Secondary builders such as the alkali metals of ethylene diamine tetraacetic acid, nitrilotriacetic acid can also be utilized in the laundry formulations of the invention. Other secondary builders known to those skilled in the art may also be utilized.

The laundry detergent formulations heretofore described may also contain additional ingredients such as enzymes, antiredeposition agents, optical brighteners, as well as dyes and perfumes known to those skilled in the art. other optional ingredients may include fabric softeners, foam suppressants, and oxygen or chlorine releasing bleaching agents.

### EXAMPLES

The following examples will serve to demonstrate the efficacy of the hydrophilic copolymer according to various embodiments of the invention. These examples should not be construed as limiting the scope of the invention.

The examples describe the various aqueous liquid detergent compositions of this invention which are stable. The numbers in each column refer to the active,- weight percentage of each component in the detergent formulation.

The nonionic surfactant used in the formulations shown in the Tables is NEODOL® 25-7, a product of Shell. The linear alkylbenzene sulfonic acid, sodium salt (LAS) was obtained from Vista under the name Vista C-560 slurry. The zeolite was "ZEOLITE A", also known as VALFOR® 100, available from the PQ Corp of Valley Forge, PA. Unless otherwise indicated, the polymer used in the formulations was a copolymer of acrylic acid with an oxyalkylated allyl alcohol, within the scope of the invention. In case of Monomer A the ratio of acrylic acid to oxyethylated allyl alcohol was 90:10 by weight, while the molar ratio was about 503:1. The molecular weight of the oxyethylated monomer was about 3800. R₁ = H, R₂ = COOM, R₃ = CH₂ - O, b = 0 and y = 0. M equals sodium in the oxyethylated monomer.

Tables 1 and 2 demonstrate the flexibility of formulating concentrated aqueous liquid detergents that allow the incorporation of major amounts of builders such as sodium citrate, sodium carbonate, and zeolite in the formulation. Furthermore, these compositions were pourable, stable compositions.

Polycarboxylates are difficult to incorporate in concentrated liquid detergents because of their incompatibility with surfactants. Example 9 in Table 3 shows that water-soluble polycarboxylates can be successfully incorporated in concentrated liquid detergent formulations that contain relatively small amounts of a copolymer according to one or more embodiments of the invention. Table 3 also illustrates several examples of detergent formulations that lack stability despite the inclusion of hydrophobically modified polymers.

**Table - 1**

| Component | Ex. 1 | Ex. 2 | Ex. 3 |
|---|---|---|---|
| LAS | 28.2 | 30 | 28.2 |
| Nonionic Surfactant | 6.6 | 7 | 6.6 |
| Sodium Citrate | 13.5 | 22 | 13.5 |
| Polymer | 1 | 1 | 0 |
| Water | 50.7 | 40 | 51.7 |
| Comment | Stable | Stable | Unstable |

**Table - 2**

| Component | Ex. 4 | Ex. 5 | Ex. 6 | Ex. 7 | Ex. 8 |
|---|---|---|---|---|---|
| LAS | 25 | 25 | 25 | 15 | 30 |
| Nonionic Surfactant | 7 | 7 | 7 | 5 | 0 |
| Sodium Citrate | | 5 | 5 | | |
| Sodium Carbonate | 15 | 8 | 8 | 8 | 15 |
| Zeolite | | 10 | 10 | 22 | |
| Lipolase | | 0.5 | | | |
| Savinase | | 0.5 | | | |
| Termamyl | | 0.5 | | | |
| Calcium Chloride | | 50 ppm | | | |
| Polymer | 1 | 1 | 1 | 1 | 1 |
| Water | 52 | 42.5 | 45 | 49 | 54 |
| Comment | Stable | Stable | Stable | Stable | Stable |

**Table - 3**

| Component | Ex. 9 | Ex. 10 | Ex. 11 | Ex. 12 | Ex. 13 |
|---|---|---|---|---|---|
| LAS | 25 | 28.3 | 30.5 | 17.43 | 28.2 |
| Nonionic Surfactant | 7 | 6.6 | 7.1 | 7 | 6.6 |
| Sodium Citrate | 5 | 13.5 | 8 | 9.33 | 13.5 |
| Sodium Carbonate | 8 | | | | |
| Zeolite | 10 | | | | |
| Sokalan® CP5 | 1.3 | | | | |
| Sokalan® PA30Cl | 1.3 | | | | |
| Sokalan® HP22 | 1.3 | | | | |
| Polymer | 1 | *1 | **0.45 | #0.88 | ##1 |
| Water | 40 | 50.7 | 53.93 | 65.39 | 50.7 |
| Comment | Stable | Unstable | Unstable | Unstable | Unstable |

| | | | | | |
|---|---|---|---|---|---|
| Lipolase, Savinase and Termamyl are laundry enzymes - Novo Nodisk BioIndustrials, Inc., Danbury, CT. * Hydrophobically modified polyether - PLURAFLO® AT 301 (BASF) | | | | | |
| ** Modified polycarboxylate - SOKALAN® HP 25 (BASF) | | | | | |
| # Maleic acid/olefin copolymer - SOKALAN® CP 9 (BASF) | | | | | |
| ## Polycarboxylate, sodium salt - SOKALAN® PA 30 CL (BASF) SOKALAN® CP5 - Acrylic acid/Maleic Acid copolymer - product of BASF. SOKALAN® PA30Cl - Polyacrylic acid, sodium salt - product of BASF SOKALAN® HP 22 - A nonionic graft copolymer - product of BASF | | | | | |

In case of Monomer B the ratio of acrylic acid to oxyalkylated allyl alcohol was 90:10 by weight, while the molar ratio was about 474:1. The oxyalkylated monomer component had a molecular weight of about 3800, and R₄ was a propyleneoxy group represented by the formula -CH₂-CH(CH₃)-O and R₅ was -CH₂-CH₂-O. In this monomer, R₁ = H, R₃ = COOM, R₃ = CH₂-O and y = 0. Also in this monomer, M = sodium.

Tables 4, 5 and 7 demonstrate the flexibility of formulating concentrated aqueous liquid detergents that allow the incorporation of major amounts of builders such as sodium citrate, sodium carbonate, and zeolite in the formulation. Furthermore, these compositions were pourable, stable compositions.

Polycarboxylates are difficult to incorporate in concentrated liquid detergents because of their incompatibility with surfactants. Example 22 in Table 6 shows that water-soluble polycarboxylates can be successfully incorporated in concentrated liquid detergent formulations that contain relatively small amounts of a copolymer according to one or more embodiments of the invention. Table 6 also illustrates several examples of detergent formulations that lack stability despite the inclusion of hydrophobically modified polymers.

**Table - 4**

| Component | Ex. 14 | Ex. 15 | Ex. 16 |
|---|---|---|---|
| LAS | 28.2 | 30 | 28.2 |
| Nonionic Surfactant | 6.6 | 7 | 6.6 |
| Sodium Citrate | 13.5 | 22 | 13.5 |
| Polymer | 1 | 1 | 0 |
| Water | 50.7 | 40 | 51.7 |
| Comment | Stable | Stable | Unstable |

**Table - 5**

| Component | Ex. 17 | Ex. 18 | Ex. 19 | Ex. 20 | Ex. 21 |
|---|---|---|---|---|---|
| LAS | 25 | 25 | 25 | 15 | 5 |
| Nonionic Surfactant | 7 | 7 | 7 | 5 | 15 |
| Sodium Citrate | 6 | 5 | 5 | | |
| Sodium Carbonate | 15 | 8 | 8 | 8 | 8 |
| Zeolite | | 10 | 10 | 22 | 22 |
| Lipolase | | 0.5 | | | |
| Savinase | | 0.5 | | | |
| Termamyl | | 0.5 | | | |
| Calcium Chloride | | 50 ppm | | | |
| Polymer | 1 | 1 | 1 | 1 | 1 |
| Water | 46 | 42.5 | 45 | 49 | 49 |
| Comment | Stable | Stable | Stable | Stable | Stable |

**Table - 6**

| Component | Ex. 22 | Ex. 23 | Ex. 24 | Ex. 25 | Ex. 26 |
|---|---|---|---|---|---|
| LAS | 25 | 28.3 | 30.5 | 17.43 | 28.2 |
| Nonionic Surfactant | 7 | 6.6 | 7.1 | 7 | 6.6 |
| Sodium Citrate | 5 | 13.5 | 8 | 9.33 | 13.5 |
| Sodium Carbonate | 8 | | | | |
| Zeolite | 10 | | | | |
| Sokalan® CP5 | 1.3 | | | | |
| Sokalan® PA30Cl | 1.3 | | | | |
| Sokalan® HP22 | 1.3 | | | | |
| Polymer | 1 | *1 | **0.45 | #0.88 | ##1 |
| Water | 40 | 50.7 | 53.93 | 65.39 | 50.7 |
| Comment | Stable | Unstable | Unstable | Unstable | Unstable |

| | | | | | |
|---|---|---|---|---|---|
| Lipolase, Savinase and Termamyl are laundry enzymes - Novo Nodisk BioIndustrials, Inc., Danbury, CT. * Hydrophobically modified polyether - PLURAFLO® AT 301 (BASF) | | | | | |
| ** Modified polycarboxylate - SOKALAN® HP 25 (BASF) | | | | | |
| # Maleic acid/olefin copolymer - SOKALAN® CP 9 (BASF) | | | | | |
| ## Polycarboxylate, sodium salt - SOKALAN® PA 30 CL (BASF) SOKALAN® CP5 -Acrylic acid/Maleic Acid copolymer - product of BASF. SOKALAN® PA30Cl -Polyacrylic acid, sodium salt - product of BASF SOKALAN® HP 22 - A nonionic graft copolymer - product of BASF | | | | | |

**Table - 7**

| Component | Ex. 27 | Ex. 28 | Ex. 29 | Ex. 30 |
|---|---|---|---|---|
| LAS | 25 | 8 | 8 | 30 |
| Nonionic Surfactant | 7 | 2 | 2 | 0 |
| Sodium Citrate | 15 | 15 | 25 | 15 |
| Polymer | 1 | 1 | 1 | 1 |
| Water | 52 | 74 | 64 | 54 |
| Comment | Stable | Stable | Stable | Stable |

## Claims

1. A stable liquid detergent composition, comprising:
a) 5 - 70% of detergent active matter selected from the group consisting of anionic, nonionic, cationic, amphoteric and zwitterionic surfactants;
b) 1 - 60% of one or more electrolytes;
c) 0.01 - 5% of at least one hydrophilic copolymer containing randomly distributed within the polymer backbone units represented by formula I or II where x, y, z, a, and b are integers and M is a alkali metal such as sodium, or hydrogen, (x + y):z is from 5:1 to 1000:1, and y can be any value ranging from zero up to the maximum value of x and b can be zero
R₁ = H or CH₃
R₂ = COOM, OCH₃, SO₃M, O-CO-CH₃, CO-NH₂
R₃ = CH₂-O-, CO-NH-
R₄ = -CH₂-CH₂-O
R₅ = alkyleneoxy group, preferably propyleneoxy or butyleneoxy groups, with the provision that the values of a and b in the sidechain are such that the combined weights of R₄ and R₅ are such that the monomer has a solubility of at least 500 grams/liter in water at 20°C;
Where R₆ = or mixtures of both, wherein in Formula II, x, y, z, a, and b are integers and M is an alkali metal such as sodium, or hydrogen, (x + y):z is from 5:1 to 1000:1, and y can be any value ranging from zero up to the maximum value of x, and b can be zero
R₁ = H or CH₃
R₂ =COOM, OCH₃, SO₃M, O-CO-CH₃, CO-NH₂
R₄ is ethyleneoxy and R₅ is alkyleneoxy, preferably propyleneoxy or butyleneoxy, with the provision that, if b is different from zero, the values of a and b in the sidechain are such that the combined weights of R₄ and R₅ are such that the monomer has a solubility of at least 500 grams/liter in water at 20°C; and
d) water; said composition having a phase separation of less than 2% over a one month period.

2. The composition as claimed in claim 1, wherein said hydrophilic copolymer is comprised of an unsaturated hydrophilic monomer copolymerized with a hydrophilic oxyalkylated monomer.

3. The composition as claimed in claim 2, wherein said unsaturated hydrophilic monomer is selected from the group consisting of acrylic acid, maleic acid, maleic anhydride, methacrylic acid, methacrylate esters and substituted methacrylate esters, vinyl acetate, methylvinyl ether and vinylsulphonate.

4. The composition as claimed in claim 2, wherein said oxyalkylated monomer is selected from the group consisting of compounds having a polymerizable olefinic moiety with at least one acidic hydrogen and are capable of undergoing addition reaction with alkylene oxide, and compounds which include monomers having at least one acidic hydrogen that are polymerized first, and then subsequently oxyalkylated.

5. The composition as claimed in claim 4, wherein said oxyalkylated monomer is the ethylene oxide adduct of allyl alcohol or the propylene oxide/ethylene oxide adduct of allyl alcohol.

6. The composition as claimed in claim 4, wherein said oxyalkylated monomer is the ethylene oxide adduct of diallylamine or the propylene oxide/ethylene oxide adduct of diallylamine.

7. The composition as claimed in claim 1, wherein the weight average molecular weight of said hydrophilic copolymer of formula I or II is in the range of 500 to 500,000.

8. The composition as claimed in claim 2, wherein said unsaturated hydrophilic monomer is acrylic acid.

9. The composition as claimed in claim 2, wherein the molar ratio of said unsaturated hydrophilic monomer to said oxyalkylated monomer is within the range of 5:1 to 1000:1.

10. The composition as claimed in claim 2, wherein the weight average molecular weight of said oxyalkylated monomer in formula I or II is within the range of 200 to 30,000.

11. A method of stabilizing a liquid detergent composition which comprises adding 0.01 - 5% by weight of at least one hydrophilic copolymer containing randomly distributed within the polymer backbone units represented by formula I or II where x, y, z, a, and b are integers and M is a alkali metal, or hydrogen, (x + y):z is from 5:1 to 1000:1, and y can be any value ranging from zero up to the maximum value of x and b can be zero
R₁ = H or CH₃
R₂ = COOM, OCH₃, SO₃M, O-CO-CH₃, CO-NH₂
R₃ = CH₂-O- CO-NH-
R₄ = -CH₂-CH₂-O
R₅ = alkyleneoxy group, preferably propyleneoxy or butyleneoxy groups, with the provision that, if b is different from zero, the values of a and b in the sidechain are such that the combined weights of R₄ and R₅ are such that the monomer has a solubility of at least 500 grams/liter in water at 20°C; where R₆ = or mixtures of both; wherein in Formula II, x, y, z, a, and b are integers and M is a alkali metal such as sodium, or hydrogen, (x + y):z is from 5:1 to 1000:1, and y can be any value ranging from zero up to the maximum value of x, and b can be zero
R₁ = H or CH₃
R₂ = COOM, OCH₃, SO₃M, O-CO-CH₃, CO-NH₂
R₄ is ethyleneoxy and R₅ is alkyleneoxy, preferably propyleneoxy or butyleneoxy, with the provision that, if b is different from zero, the values of a and b in the sidechain are such that the combined weights of R₄ and R₅ are such that the monomer has a solubility of at least 500 grams/liter in water at 20°C.

12. The method as claimed in claim 11, wherein said hydrophilic copolymer is comprised of an unsaturated hydrophilic monomer copolymerized with a hydrophilic oxyalkylated monomer.

13. The method as claimed in claim 12, wherein said unsaturated hydrophilic monomer is selected from the group consisting of acrylic acid, maleic acid, maleic anhydride, methacrylic acid, methacrylate esters and substituted methacrylate esters, vinyl acetate, methylvinyl ether, and vinylsulphonate.

14. The method as claimed in claim 12, wherein said oxyalkylated monomer is selected from the group consisting of compounds having a polymerizable olefinic moiety with at least one acidic hydrogen and are capable of undergoing addition reaction with alkylene oxides, and compounds which include monomers having at least one acidic hydrogen that are polymerized first, and then subsequently oxyalkylated.

15. The method as claimed in claim 12, wherein said oxyalkylated monomer is the ethylene oxide adduct of allyl acohol or the propylene oxide/ethylene oxide adduct of allyl alcohol.

16. The method as claimed in claim 14, wherein said oxyalkylated monomer is the ethylene oxide adduct of diallylamine or the propylene oxide/ethylene oxide adduct of diallylamine.

17. The method as claimed in claim 11, wherein the weight average molecular weight of said hydrophilic copolymer of formula I or II is in the range of 500 to 500,000.

## Patentansprüche

1. Stabile Flüssigwaschmittelzusammensetzung, enthaltend:
a) 5-70% waschaktive Substanzen aus der Gruppe bestehend aus anionischen, nichtionischen, kationischen, amphoteren und zwitterionischen Tensiden;
b) 1-60% eines oder mehrerer Elektrolyte;
c) 0,01-5% mindestens eines hydrophilen Copolymers, das in den Polymerhauptketten in statistischer Verteilung Einheiten der Formel I oder II worin x, y, z, a und b ganze Zahlen sind und M für ein Alkalimetall, wie Natrium, oder Wasserstoff steht, (x+y):z im Bereich von 5:1 bis 5000:1 liegt, y ein beliebiger Wert im Bereich von Null bis zum Höchstwert von x und b gleich Null sein kann,
R₁ = H oder CH₃,
R₂ = COOM, OCH₃, SO₃M, O-CO-CH₃, CO-NH₂,
R₃ = CH₂-O-, CO-NH-
R₄ = -CH₂-CH₂-O
R₅ = Alkylenoxygruppe, bevorzugt Propylenoxy- oder Butylenoxygruppen, mit der Maßgabe, daß a und b in der Seitenkette solche Werte haben, daß das Gesamtgewicht von R₄ und R₅ so groß ist, daß das Monomer eine Wasserlöslichkeit von mindestens 500 Gramm/Liter bei 20°C aufweist;
worin R₆ = oder Gemische davon enthält, wobei in Formel II x, y, z, a und b ganze Zahlen sind und M für ein Alkalimetall, wie Natrium, oder Wasserstoff steht, (x+y):z im Bereich von 5:1 bis 5000:1 liegt, y ein beliebiger Wert im Bereich von Null bis zum Höchstwert von x und b gleich Null sein kann,
R₁ = H oder CH₃,
R₂ = COOM, OCH₃, SO₃M, O-CO-CH₃, CO-NH₂,
R₄ für Ethylenoxy und R₅ für Alkylenoxy, bevorzugt Propylenoxy oder Butylenoxy, steht, mit der Maßgabe, daß, wenn b nicht gleich Null ist, a und b in der Seitenkette solche Werte haben, daß das Gesamtgewicht von R₄ und R₅ so groß ist, daß das Monomer eine Wasserlöslichkeit von mindestens 500 Gramm/Liter bei 20°C aufweist;
und
d) Wasser; wobei die Zusammensetzung über einen Zeitraum von einem Monat weniger als 2% Phasentrennung aufweist.

2. Zusammensetzung nach Anspruch 1, bei der das hydrophile Copolymer aus einem mit einem hydrophilen oxyalkylierten Monomer copolymerisierten, ungesättigten hydrophilen Monomer aufgebaut ist.

3. Zusammensetzung nach Anspruch 2, bei der das ungesättigte hydrophile Monomer aus der Gruppe bestehend aus Acrylsäure, Maleinsäure, Maleinsäureanhydrid, Methacrylsäure, gegebenenfalls substituierten Methacrylsäureestern, Vinylacetat, Methylvinylether und Vinylsulfonat stammt.

4. Zusammensetzung nach Anspruch 2, bei der das oxyalkylierte Monomer aus der Gruppe bestehend aus Verbindungen, die eine polymerisierbare olefinische Gruppierung mit mindestens einem sauren Wasserstoffatom enthalten und Additionsreaktionen mit Alkylenoxid eingehen können, und Verbindungen, die Monomere mit mindestens einem sauren Wasserstoffatom enthalten und zunächst polymerisiert und anschließend oxyalkyliert werden, stammt.

5. Zusammensetzung nach Anspruch 4, bei der es sich bei dem oxyalkylierten Monomer um das Ethylenoxid-Addukt von Allylalkohol oder das Propylenoxid/Ethylenoxid-Addukt von Allylalkohol handelt.

6. Zusammensetzung nach Anspruch 4, bei der es sich bei dem oxyalkylierten Monomer um das Ethylenoxid-Addukt von Diallylamin oder das Propylenoxid/Ethylenoxid-Addukt von Diallylamin handelt.

7. Zusammensetzung nach Anspruch 1, bei der das gewichtsmittlere Molekulargewicht des hydrophilen Copolymers der Formel I oder II im Bereich von 500 bis 500.000 liegt.

8. Zusammensetzung nach Anspruch 2, bei der es sich bei dem ungesättigten hydrophilen Monomer um Acrylsäure handelt.

9. Zusammensetzung nach Anspruch 2, bei der das Molverhältnis von ungesättigtem hydrophilem Monomer zu oxyalkyliertem Monomer im Bereich von 5:1 bis 1000:1 liegt.

10. Zusammensetzung nach Anspruch 2, bei der das gewichtsmittlere Molekulargewicht des oxyalkylierten Monomers in Formel I oder II im Bereich von 200 bis 30.000 liegt.

11. Verfahren zur Stabilisierung einer Flüssigwaschmittelzusammensetzung, bei dem man 0,01-5 Gew.-% mindestens eines hydrophilen Copolymers, das in den Polymerhauptketten in statistischer Verteilung Einheiten der Formel I oder II worin x, y, z, a und b ganze Zahlen sind und M für ein Alkalimetall oder Wasserstoff steht, (x+y):z im Bereich von 5:1 bis 1000:1 liegt, y ein beliebiger Wert im Bereich von Null bis zum Höchstwert von x und b gleich Null sein kann,
R₁ = H oder CH₃,
R₂ = COOM, OCH₃, SO₃M, O-CO-CH₃, CO-NH₂,
R₃ = CH₂-O-, CO-NH-
R₄ = -CH₂-CH₂-O
R₅ = Alkylenoxygruppe, bevorzugt Propylenoxy- oder Butylenoxygruppen, mit der Maßgabe, daß, wenn b nicht gleich Null ist, a und b in der Seitenkette solche Werte haben, daß das Gesamtgewicht von R₄ und R₅ so groß ist, daß das Monomer eine Wasserlöslichkeit von mindestens 500 Gramm/Liter bei 20°C aufweist; worin R₆ = oder Gemische davon enthält, wobei in Formel II x, y, z, a und b ganze Zahlen sind und M für ein Alkalimetall, wie Natrium, oder Wasserstoff steht, (x+y):z im Bereich von 5:1 bis 1000:1 liegt, y ein beliebiger Wert im Bereich von Null bis zum Höchstwert von x und b gleich Null sein kann,
R₁ = H oder CH₃,
R₂ = COOM, OCH₃, SO₃M, O-CO-CH₃, CO-NH₂,
R₄ für Ethylenoxy und R₅ für Alkylenoxy, bevorzugt Propylenoxy oder Butylenoxy, steht, mit der Maßgabe, daß, wenn b nicht gleich Null ist, a und b in der Seitenkette solche Werte haben, daß das Gesamtgewicht von R₄ und R₅ so groß ist, daß das Monomer eine wasserlöslichkeit von mindestens 500 Gram/Liter bei 20°C aufweist,
zusetzt.

12. Verfahren nach Anspruch 11, bei dem man ein hydrophiles Copolymer einsetzt, das aus einem mit einem hydrophilen oxyalkylierten Monomer copolymerisierten, ungesättigten hydrophilen Monomer aufgebaut ist.

13. Verfahren nach Anspruch 12, bei dem man das ungesättigte hydrophile Monomer aus der Gruppe bestehend aus Acrylsäure, Maleinsäure, Maleinsäureanhydrid, Methacrylsäure, gegebenenfalls substituierten Methacrylsäureestern, Vinylacetat, Methylvinylether und Vinylsulfonat auswählt.

14. Verfahren nach Anspruch 12, bei dem man das oxyalkylierte Monomer aus der Gruppe bestehend aus Verbindungen, die eine polymerisierbare olefinische Gruppierung mit mindestens einem sauren Wasserstoffatom enthalten und Additionsreaktionen mit Alkylenoxiden eingehen können, und Verbindungen, die Monomere mit mindestens einem sauren Wasserstoffatom enthalten und zunächst polymerisiert und anschließend oxyalkyliert werden, auswählt.

15. Verfahren nach Anspruch 12, bei dem man als oxyalkyliertes Monomer das Ethylenoxid-Addukt von Allylalkohol oder das Propylenoxid/Ethylenoxid-Addukt von Allylalkohol einsetzt.

16. Verfahren nach Anspruch 14, bei dem man als oxyalkyliertes Monomer das Ethylenoxid-Addukt von Diallylamin oder das Propylenoxid/Ethylenoxid-Addukt von Diallylamin einsetzt.

17. Verfahren nach Anspruch 11, bei dem man ein hydrophiles Copolymer der Formel I oder II mit einem gewichtsmittleren Molekulargewicht im Bereich von 500 bis 500.000 einsetzt.

## Revendications

1. Composition détergente liquide stable, comprenant:
a) 5 à 70% de substance active détergente choisie dans le groupe formé par les tensio-actifs anioniques, non ioniques, cationiques, amphotériques et zwittérioniques;
b) 1 à 60% d'un ou plusieurs électrolytes;
c) 0,01 à 5% d'au moins un copolymère hydrophile, contenant aléatoirement distribués dans de squelette polymère, des motifs représentés par la formule I ou II: où x, y, z, a et b sont des nombres entiers et M est un métal alcalin tel que le sodium ou un atome d'hydrogène, (x+y):z est de 5:1 à 1 000:1, et y peut être toute valeur comprise entre zéro jusqu'à la valeur maximale de x et b peut être nul
R₁ = H ou CH₃;
R₂ = COOM, OCH₃, SO₃M, O-CO-CH₃, CO-NH₂
R₃ = CH₂-O-, CO-NH-
R₄ = -CH₂-CH₂-O
R₅ = un groupe alkylénoxy, de préférence les groupes propylénoxy ou butylénoxy, à condition que les valeurs de a et b dans la chaîne latérale soient telles que les masses combinées de R₄ et R₅ sont telles que le monomère possède une solubilité d'au moins 500 grammes/litre dans l'eau à 20°C;
où R₆ = ou des mélanges des deux, dans lesquels dans la formule II, x, y, z, a et b sont des nombres entiers et M est un métal alcalin tel que le sodium, ou un atome d'hydrogène, (x + y):z vaut de 5:1 à 1 000:1, et y peut être toute valeur allant de zéro jusqu'à la valeur maximale de x, et b peut être nul;
R₁ = H ou CH₃;
R₂ = COOM, OCH₃, SO₃M, O-CO-CH₃, CO-NH₂;
R₄ est un groupe éthylénoxy et R₅ est un groupe alkylénoxy, de préférence propylénoxy ou butylénoxy, à condition que, si b est différent de zéro, les valeurs de a et b dans la chaîne latérale soient telles que les masses combinées de R₄ et R₅ sont telles que le monomère a une solubilité d'au moins 500 grammes/litre dans l'eau à 20°C; et
d) de l'eau; ladite composition ayant une séparation de phase inférieure à 2% pendant une durée d'un mois.

2. Composition selon la revendication 1, dans laquelle ledit copolymère hydrophile est composé d'un monomère hydrophile insaturé copolymérisé avec un monomère oxyalkylé hydrophile.

3. Composition selon la revendication 2, dans laquelle ledit monomère hydrophile insaturé est choisi dans le groupe formé par l'acide acrylique, l'acide maléique, l'anhydride maléique, l'acide méthacrylique, les esters méthacrylate et les esters méthacrylate substitués, l'acétate de vinyle, l'éther méthylvinylique et le vinylsulfonate.

4. Composition selon la revendication 2, dans laquelle ledit monomère oxyalkylé est choisi dans le groupe formé par les composés ayant une fraction oléfinique polymérisable avec au moins un hydrogène acide et qui sont capables de subir une réaction d'addition avec un oxyde d'alkylène, et les composés qui incluent des monomères ayant au moins un hydrogène acide qui sont polymérisés d'abord, puis ultérieurement oxyalkylés.

5. Composition selon la revendication 4, dans laquelle ledit monomère oxyalkylé est le produit d'addition d'oxyde d'éthylène et d'alcool allylique ou le produit d'addition d'oxyde de propylène/oxyde d'éthylène et d'alcool allylique.

6. Composition selon la revendication 4, dans laquelle ledit monomère oxyalkylé est le produit d'addition d'oxyde d'éthylène et de diallylamine ou le produit d'addition d'oxyde de propylène/oxyde d'éthylène et de diallylamine.

7. Composition selon la revendication 1, dans laquelle la masse moléculaire moyenne en masse dudit copolymère hydrophile de formule I ou II est dans la gamme de 500 à 500 000.

8. Composition selon la revendication 2, dans laquelle le monomère hydrophile insaturé est l'acide acrylique.

9. Composition selon la revendication 2, dans laquelle le rapport molaire dudit monomère hydrophile insaturé audit monomère oxyalkylé est dans la gamme de 5:1 à 1 000:1.

10. Composition selon la revendication 2, dans laquelle la masse moléculaire moyenne en masse dudit monomère oxyalkylé dans la formule I ou II est dans la gamme de 200 à 30 000.

11. Procédé pour stabiliser une composition détergente liquide qui consiste à ajouter 0,01 à 5% en poids d'au moins un copolymère hydrophile, contenant aléatoirement distribué dans le squelette polymère, des motifs représentés par la formule I ou II: où x, y, z, a et b sont des nombres entiers et M est un métal alcalin ou un atome d'hydrogène, (x+y):z vaut de 5:1 à 1 000:1, et y peut être toute valeur allant de zéro jusqu'à la valeur maximale de x, et b peut être nul
R₁ = H ou CH₃;
R₂ = COOM, OCH₃, SO₃M, O-CO-CH₃, CO-NH₂
R₃ = CH₂-O-, CO-NH-
R₄ = -CH₂-CH₂-O
R₅ = un groupe alkylénoxy, de préférence les groupes propylénoxy ou butylénoxy, à condition que, si b est différent de zéro, les valeurs de a et b dans la chaîne latérale soient telles que les masses combinées de R₄ et R₅ sont telles que le monomère possède une solubilité d'au moins 500 grammes/litre dans l'eau à 20°C;
où R₆ = ou des mélanges des deux, dans lesquels dans la formule II, x, y, z, a et b sont des nombres entiers et M est un métal alcalin tel que le sodium, ou un atome d'hydrogène, (x + y):z vaut de 5:1 à 1 000:1, et y peut être toute valeur allant de zéro jusqu'à la valeur maximale de x, et b peut être nul;
R₁ = H ou CH₃;
R₂ = COOM, OCH₃, SO₃M, O-CO-CH₃, CO-NH₂;
R₄ est un groupe éthylénoxy et R₅ est un groupe alkylénoxy, de préférence propylénoxy ou butylénoxy, à condition que, si b est différent de zéro, les valeurs de a et b dans la chaîne latérale soient telles que les masses combinées de R₄ et R₅ sont telles que le monomère a une solubilité d'au moins 500 grammes/litre dans l'eau à 20°C.

12. Procédé selon la revendication 11, dans lequel ledit copolymère hydrophile est composé d'un monomère hydrophile insaturé copolymérisé avec un monomère oxyalkylé hydrophile.

13. Procédé selon la revendication 12, dans lequel ledit monomère hydrophile insaturé est choisi dans le groupe formé par l'acide acrylique, l'acide maléique, l'anhydride maléique, l'acide méthacrylique, les esters méthacrylate et les esters méthacrylate substitués, l'acétate de vinyle, l'éther méthylvinylique et le vinylsulfonate.

14. Procédé selon la revendication 12, dans lequel ledit monomère oxyalkylé est choisi dans le groupe formé par les composés ayant une fraction oléfinique polymérisable avec au moins un hydrogène acide et qui sont capables de subir une réaction d'addition avec les oxydes d'alkylène, et les composés qui incluent des monomères ayant au moins un hydrogène acide qui sont polymérisés d'abord, puis ultérieurement oxyalkylés.

15. Procédé selon la revendication 12, dans lequel ledit monomère oxyalkylé est le produit d'addition d'oxyde d'éthylène et d'alcool allylique ou le produit d'addition d'oxyde de propylène/oxyde d'éthylène et d'alcool allylique.

16. Procédé selon la revendication 14, dans lequel ledit monomère oxyalkylé est le produit d'addition d'oxyde d'éthylène et de diallylamine ou le produit d'addition d'oxyde de propylène/oxyde d'éthylène et de diallylamine.

17. Procédé selon la revendication 11, dans lequel la masse moléculaire moyenne en masse dudit copolymère hydrophile de formule I ou II est dans la gamme de 500 à 500 000.
